

## UNITED STATES PATENT OFFICE

2,200,839

WATER-RESISTANT LAMINATED PAPER  
AND METHOD OF MANUFACTURELouis C. Fleck, Appleton, Wis., assignor to Paper  
Patents Company, Neenah, Wis., a corporation  
of WisconsinNo Drawing. Application June 29, 1936,  
Serial No. 87,952

6 Claims. (Cl. 154—40)

The present invention relates to laminated paper and the method of preparing the same. More particularly, the present invention relates to paper sheets bonded together with a water-resistant binding composition. The laminated paper prepared in accordance with the present invention has been found particularly adapted for use in the manufacturing of embossed wall paper.

When regular embossed wall paper is hung on the wall by the paper hanger, practically all of the relief present and produced by the embossing operation will be found to have flattened out as soon as the paper has dried. This unsatisfactory result is caused primarily by the fact that in the ordinary process of paper hanging the back of the paper is first covered with a starch paste which is allowed to soak into the paper for several minutes before applying the paper to the wall. During this period in which the paste is soaking into the paper, the paper becomes very soft and pliable so that, when hung on the wall and rolled or brushed down tight, most of the relief of the embossing is flattened out and the embossing effect largely lost.

I have found that a more permanent embossing effect can be maintained after the paper is hung on the wall if the paper employed, instead of being the ordinary single ply, is made up of a laminated paper consisting of two sheets pasted or bonded together with a water-proof film or glue. The laminated papers heretofore available have not, however, been found entirely satisfactory. For example, paper bonded with water-proof adhesives including latex, cellulose ethers and esters, asphalt combinations, and the so-called water-proof animal glues, were objectionable due either to high cost, change in color, or difficulty of application.

It is an object of my invention to prepare a laminated paper employing a water-proof bonding composition that does not change in color. It is also an object of my invention to prepare a laminated paper employing a water-proof bonding composition that is not difficult of application.

It is a further object of my invention to produce a laminated paper employing a low cost water-proof bonding composition that is particularly suitable for use in making embossed wall paper.

I have discovered that an improved laminated paper having the desired characteristics may be made by treating one side of a sheet of paper with an alkaline solution of a potentially water-

resistant protein adhesive; treating one side of a second sheet of paper with a starch-like adhesive containing an agent adapted to render the protein adhesive water-resistant, and pressing the treated sides of the sheets together.

The following example employing twelve ounce wall paper will serve to illustrate my invention.

The bonding composition or glue which is used to bind the paper together is of course made up in separate parts, one part of the glue being applied to the first or bottom sheet and the other part to the second or top sheet just prior to the pressing of the two sheets together. The first part of the glue, which may be applied to the first or bottom sheet, may be made up of a formula as follows.

|                                        | Parts |
|----------------------------------------|-------|
| Soya bean flour                        | 450   |
| Water                                  | 1750  |
| Borax dissolved in 1000 parts of water | 45    |
| Phenol                                 | 22.5  |

In the preparation of this adhesive the soya bean flour is first mixed with enough water to form a thick paste and then cut with an alkali such as borax dissolved in water at about 50° C. according to the usual practice in wall paper mills. The rest of the water and phenol are then added and this part of the glue is ready for use.

The second part of the glue which may be applied to the second or top sheet is made by cooking one part of a starch-like adhesive such as tapioca flour mixed with 19.5 parts of water to about 75-80° C. according to the general methods used in wall paper mills. To this material is added slowly with stirring about 18 parts of commercial formalin, i. e. an aqueous solution of formaldehyde. After cooling the starch formaldehyde adhesive is ready for application.

In place of the borax and soya bean flour, other alkalis and other alkali-soluble potentially water-resistant proteins such as casein may be used. Although the presence of the phenol is optional, the addition of phenol and like substances that react with formaldehyde have been found advantageous as they add to the water-resistance of the bonded papers. In place of the tapioca flour, which acts as a carrier for the insolubilizing agent, other starch-like adhesives may be used. The formaldehyde insolubilizing agent may be partially or totally replaced by aluminum salts such as alum (aluminum sulphate) and aluminum formate. The protein adhesive may also contain resins which will in-

solubilize when combined with aluminum salts carried by the starch. The starch adhesive may also serve as a carrier for flexibilizing agents such as glycerol.

5. In the operation of applying the respective adhesives to the top and bottom sheets and making a laminated sheet from the same, the two rolls of paper consisting of the top and the bottom sheets respectively, are mounted on separate unwinding stands. The paper from each unwinding stand then passes over a machine in which each sheet of paper receives a coating of its respective adhesive. This machine may be a reverse roll coater, a blotch roller, or a brush coater. It is understood that there is a separate treating machine for each sheet, the protein adhesive being applied, for example, to one side of the bottom sheet and the starch adhesive being applied to one side of the top sheet. From the machines the respective sheets pass over a doctor bar or scraper knife which scrapes off all the excess adhesive which might be piled upon the paper leaving only a very thin film of adhesive on the surface and some adhesive which has already penetrated into the sheet. After passing over the scraper knives, the two sheets then are run together so that the treated sides are next to each other and in this position the two sheets travel to rollers and are pressed together in the usual manner. If the paper is to be embossed, it travels directly to the embosser, which presses the sheets firmly together at the same time that the embossing is done. The sequence of operation described above is continuous, the whole operation of applying the adhesive, scraping off the excess, and pressing the sheets together, taking place in a period of a few seconds. The embossing of the somewhat soft, freshly treated paper before the adhesive layer has dried out and completely set to a water-resistant layer, is the preferred procedure when the paper is to be embossed.

The laminated paper prepared by my process is water-resistant and when embossed retains its relief even when subjected to the most severe of paper hanging treatments. Although the embossing effect is not brushed or flattened out by the paper hanger when soaked with starch paste and hung on the wall, the paper nevertheless becomes pliable and workable for hanging. The laminated sheets bonded with my low cost bonding composition, which is simple in application, are not subject to color change and are durable when exposed or stored in warm, damp places under conditions which tend to promote growth of mold and other micro organisms.

Although I have stressed the use of my laminated paper for use in making embossed wall paper, it will be understood that my paper may be used for wrapping paper boxes and for all other like uses, and particularly where water-resistant, durable paper not subjected to color change is desired. It will also be understood that while I have illustrated my invention showing the

use of specific compositions, my invention is not limited thereto, as all modifications coming within the true spirit and scope of my invention are intended to be covered by the claims appended hereto.

I claim:

1. A method of preparing laminated paper particularly adapted for use in the manufacture of embossed wall paper comprising treating one side of a sheet of paper with an alkaline solution of a potentially water-resistant casein adhesive, treating one side of a second sheet of paper with a starch adhesive containing an agent adapted to render said casein adhesive water-resistant, and pressing the freshly treated sides of said sheets together.

2. A method of preparing embossed laminated paper comprising treating one side of a sheet of paper with an alkaline solution of a potentially water-resistant casein adhesive, treating one side of a second sheet of paper with a starch adhesive containing an agent adapted to render said casein adhesive water-resistant, and simultaneously embossing said laminated paper while pressing the freshly treated sides of said sheets together.

3. A method of preparing laminated paper comprising treating one side of a sheet of paper with an alkaline solution of a potentially water-resistant casein adhesive, treating one side of a second sheet of paper with a starch adhesive containing formaldehyde, and pressing the freshly treated sides of said sheets together.

4. A method of preparing laminated paper comprising treating one side of a sheet of paper with an alkaline solution of a potentially water-resistant casein adhesive, treating one side of a second sheet of paper with a starch adhesive containing salts of aluminum selected from the group consisting of aluminum sulphate and aluminum formate, and pressing the freshly treated sides of said sheets together.

5. Laminated paper particularly adapted for use as embossed wall paper comprising two sheets of paper cemented together with a casein adhesive and a starch adhesive containing a casein insolubilizing agent selected from the group comprising formaldehyde and soluble aluminum salts selected from the group consisting of aluminum sulphate and aluminum formate.

6. A method of preparing laminated paper comprising treating one side of the sheet of paper with a potentially water-resistant casein adhesive containing a small amount of phenol, treating one side of a second sheet of paper with a starch adhesive containing formaldehyde, and pressing the treated sides of said sheets together, sufficient formaldehyde being present to insolubilize the casein adhesive and react with the phenol, the amount of phenol being effective to provide a substantial increase in water resistance of said laminated paper.

LOUIS C. FLECK.